# NEW EUROPEAN PATENT SPECIFICATION

(11) **EP 1 109 845 B2**
(45) Date of publication and mention of the opposition decision: **22.09.2010**
(45) Mention of the grant of the patent: 19.10.2005
(21) Application number: 99942005.2
(22) Date of filing: 06.08.1999
(51) Int. Cl.: C08F 220/34, D06M 15/21

(54) **NOVEL LATEX COMPOSITIONS FOR DEPOSITION ON VARIOUS SUBSTRATES**
NEUE LATEX ZUSAMMENSETZUNG FÜR BESCHICHTUNG VON VERSCHIEDENEN SUBSTRATEN
NOUVELLES COMPOSITIONS A BASE DE LATEX DESTINEES A ETRE DEPOSEES SUR DIVERS SUBSTRATS

(30) Priority: 07.08.1998 US 95660 P
(43) Date of publication of application: 27.06.2001
(73) Proprietor: Reichhold Inc., Durham, NC 27703 (US)
(72) Inventor: KRISHNAN, Venkataram, Cary, NC 27513 (US)
(74) Representative: Harrison Goddard Foote
(86) International application number: PCT/US1999/017670
(87) International publication number: WO 2000/008077

(56) References cited:
- EP-A- 0 000 426
- EP-A- 0 239 213
- EP-A- 0 286 009
- EP-A- 0 469 196
- EP-A- 0 747 456
- WO-A-97/15603
- WO-A-98/51720
- WO-A-97//45468
- DE-A- 3 339 662
- GB-A- 1 299 012
- US- - 4 617 343
- US-A- 4 226 748
- US-A- 5 247 008
- US-A- 5 403 640
- US-A- 5 447 643
- US-A- 5 608 021
- DATABASE CHEMABS [Online] CHEMICAL ABSTRACTS SERVICE, COLUMBUS, OHIO, US NAPPER, D. H.: "Steric stabilization" retrieved from STN Database accession no. 86:107053 XP002125110 & J. COLLOID INTERFACE SCI. ( 1977 ), 58(2), 390-407 ,
- 'Römpp Chemie Lexikon', vol. 5, 1995, GEORG THIEME VERLAG, NEW YORK pages 3558 - 3559

## Description

### Cross-Reference to Related Applications

The instant application claims priority to U.S. Provisional Application Serial No. 60/095,660 filed 7 August 1998.

### Field and Background of the Invention

The invention generally relates to polymer latices, and is especially concerned with polymer latices which may be uniformly deposited onto the surface of a substrate.

The deposition of polymer latices on solid substrates (e.g., inorganic or organic fillers, pigments, particles) has been known for some time so as to impart certain end use performance properties such as, for example, hydrophobicity, strength and compatibility to the substrates. The polymer latices have typically been anionic, but cationic latices have also been used. Anionic polymer latices may be deposited on negatively-charged fibers by using a retention aid (e.g., alum or a water-soluble cationic polymer). A water-soluble cationic polymer may be employed since it is able to facilitate the deposition of the latex onto a fiber surface. The process of using a retention aid involves depositing an anionic latex onto fibers which are typically cellulosic or wood fibers. This process is known as beater addition. For the most part, the beater addition process generally depends on the flocculation of an anionic latex on fibers through the use of the retention aid. Another process for depositing anionic polymer latices on fibers is known as the saturation process. In this saturation process, a premade fiber web is saturated with the anionic latex.

Several problems exist with respect to the above procedures. With respect to the beater addition process, the latex is flocculated on the fibers in an indiscrete manner, and as a result physical properties relating to strength, resiliency, water repellency, and surface coverage may not be sufficiently imparted to a fibrous structure such as a mat or composite made therefrom. With respect to the saturation process, the coating of the fibers is typically inefficient since the anionic latex often does not uniformly cover the fibers. As a result, a sizeable quantity of latex may be needed to penetrate and saturate the fiber web. Moreover, because the deposition of the anionic latex is often non-uniform, physical properties may not be consistent throughout the fiber web. This physical property inconsistency may become magnified at low latex add-on levels.

As referred to above, it has also been known to deposit cationic polymer latices on fiber surfaces. These cationic polymer latices usually contain low molecular weight cationic surfactants. The use of these surfactants, however, is becoming less desirable due to heightened environmental concerns. In particular, the surfactants may be potentially toxic in aquatic systems.

In view of the above, it is an object of the present invention to provide a cationic polymer latex for deposition on a fiber surface which addresses the problems noted above. In particular, it would be desirable to obviate the need for using retention aids and conventional cationic surfactants in the deposition of cationic polymer latices on fibers. Moreover, it would be desirable if the cationic polymer latex used in the deposition could be employed in relatively low amounts.

### Summary of the Invention

In one aspect, the invention provides a cationic polymer latex composition formed by emulsion polymerisation. The latex composition comprises an ethylenically unsaturated monomer, an ethylenically unsaturated cationic monomer, a monomer possessing alkoxylated functionality incorporated into the cationic polymer latex to provide steric stabilization and a free radical initiator. The cationic polymer latex composition preferably has a solids content of no less than 35 weight percent solids, and more preferably no less than 40 weight percent solids.

### Detailed Description of the Preferred Embodiment

The invention will now be described in greater detail with respect to the embodiments and examples illustrated hereinbelow.

Various ethylenically unsaturated monomers may be used in the latex. Examples of monomers can be found in U.S. Patent No. 5,830,934 to Krishnan, the disclosure of which is incorporated herein by reference in its entirety. Such monomers include, but are not limited to, vinyl aromatic monomers (e.g., styrene, para methyl styrene, chloromethyl styrene, vinyl toluene); olefins (e.g., ethylene); aliphatic conjugated diene monomers (e.g., butadiene); non-aromatic unsaturated mono- or dicarboxylic ester monomers (e.g., methyl methacrylate, ethyl acrylate, butyl acrylate, butyl methacrylate, glycidyl methacrylate, isodecyl acrylate, lauryl acrylate); monomers based on the half ester of an unsaturated dicarboxylic acid monomer (e.g., monomethyl maleate); unsaturated mono- or dicarboxylic acid monomers and derivatives thereof (e.g., itaconic acid); and nitrogen-containing monomers (e.g., acrylonitrile, methacrylonitrile, acrylamide, methacrylamide, N-methylol acrylamide, N-(isobutoxymethyl) acrylamide); vinyl ester monomers which includes branched vinyl esters (e.g., vinyl neodecanoate, vinyl versatates), and monomers containing ethylenic unsaturation such as vinyl acetate. Fluorinated analogs of alkyl acrylates or methacrylates may also be used. Mixtures of the above may be used.

The latex preferably comprises from 70 to 99 percent of the ethylenically unsaturated monomer based on the total monomer weight.

The latex also includes an ethylenically unsaturated cationic monomer. For the purposes of the invention, the term "cationic monomer" refers to any monomer which possesses a net positive charge. This positive charge may be imparted by a heteroatom which is present in the monomer. Exemplary heteroatoms include nitrogen, sulfur, and phosphorus. The cationic monomer is incorporated into the latex polymer by virtue of its ethylenic unsaturation. Examples of cationic monomers include amine and amide monomers, and quaternary amine monomers. Amine and amide monomers include: dimethylaminoethyl acrylate; diethylaminoethyl acrylate; dimethyl aminoethyl methacrylate; diethylaminoethyl methacrylate; tertiary butylaminoethyl methacrylate; N,N-dimethyl acrylamide; N,N-dimethylaminopropyl acrylamide; acryloyl morpholine; N-isopropyl acrylamide; N,N-diethyl acrylamide; dimethyl aminoethyl vinyl ether; 2-methyl-1-vinyl imidazole; N,N-dimethyl- aminopropyl methacrylamide; vinyl pyridine; vinyl benzyl amine; and mixtures thereof.

Quaternary amine monomers which may be used in the latex of the invention can include those obtained from the above amine monomers such as by protonation using an acid or via an alkylation reaction using an alkyl halide. Examples of quaternary amine monomers include, but are not limited to: dimethylaminoethyl acrylate, methyl chloride quarternary; dimethylaminoethyl methacrylate, methyl chloride quarternary; diallyldimethylammonium chloride; N,N-dimethylaminopropyl acrylamide, methyl chloride quaternary; trimethyl-(vinyloxyethyl) ammonium chloride; 1-vinyl-2,3-dimethylimidazolinium chloride; vinyl benzyl amine hydrochloride; and vinyl pyridinium hydrochloride. Mixtures of the above may also be used.

Amine salts can also be used and are obtained, for example, by the reaction of an epoxy group with a secondary amine and subsequent neutralization of the newly formed tertiary amine with an acid. An.example of this is the reaction product of glycidyl methacrylate with a secondary amine that can be free radically polymerized. Quaternary amine functionality can also be generated as a post reaction on a preformed polymer having, for example, an epoxy group. Examples of these kinds of reactions are described in the article, "Polymer Compositions for Cationic Electrodepositable Coatings, Journal of Coatings Technology, Vol 54, No 686, March 1982. It should also be appreciated that cationic functionality can also be imparted via sulfonium or phosphonium chemistry examples of which are described in the above article.

The latex preferably comprises from about 0.5 to about 15 percent of the cationic monomer based on the total monomer weight.

The latex also comprises a component which is incorporated into the cationic polymer latex to sterically stabilize the latex. Suitable components include monomers, as set forth below. For the purposes of the invention, the term "incorporated" with respect to the use of the monomer means that the monomer attaches to the backbone of the cationic polymer. This stabilizing component is a nonionic monomer which incorporates steric stabilization to the latex particle without affecting the deposition characteristics of the cationic polymer latex and which contains alkoxylated (e.g., ethoxylated or propoxylated) functionality. Examples of such monomers include those described by the formulas: (a) CH₂=C(R)COO(CH₂CHR'O)ₙR"-- where R=H, C₁-C₄ alkyl; and R'= H, C₁-C₄ alkyl, and R"= H, C₁-C₄ alkyl, and n=1-30; (b) CH₂=C(R)COO(CH₂CH₂O)ₙ(CH₂CHR'O)ₘR"-- where R= H, C₁-C₄ alkyl, and R'= H, C₁-C₄ alkyl, and R"= H, C₁-C4 alkyl, n and m each may range from 1-15; and (c) CH₂=C(R)COO(CH₂CHR'O)ₙ(CH₂CH₂O)ₘR"-- where R= H, C₁-C₄ alkyl, and R'=H, C₁-C₄ alkyl and R"= H, C₁-C₄ alkyl, n and m = 1-15. Preferably, CH₃ is employed for the above ranges defined by C₁-C₄ alkyl.

Ethoxylated mono- and diesters of diacids such as maleic and itaconic acids can also be used to achieve the same stabilizing effect. Also acrylate, methacrylate, vinyl and allyl versions of surfactants or polymerizable surfactants as they are commonly named can also be used. Examples of these are TREM LF-40 sold by Henkel of Düsseldorf, Germany, and SAM 186 N sold by BASF of Mount Olive, New Jersey. These surfactants are characteristic in that they possess ethylenic unsaturation that allows the surfactants to be incorporated into the latex polymer. Similar to other surfactants, these materials have hydrophobic and hydrophilic functionality that varies. Surfactants that are particularly applicable to the present invention are nonionic surfactants wherein the hydrophilic character is believed to be attributable to the presence of alkylene oxide groups (eg: ethylene oxide, propylene oxide and butylene oxide). The degree of hydrophilicity can vary based on the selection of functionality.

The component which is used to stabilize the latex is present in an amount ranging from 0.5 to 15 percent based on the total weight of the monomers.

The latex of the invention also includes a free radical initiator, the selection of which is known in the art. Preferably, a free radical initiator is used which generates a cationic species upon decomposition and contributes to the cationic charge of the latex. An example of such an initiator is 2,2'-azobis(2-amidinopropane) dihydrochloride) sold commercially as Wako V-50 by Wako Chemicals of Richmond, Virginia.

The latex of the invention may also include other additives to improve the physical and/or mechanical properties of the polymer, the selection of which are known to one skilled in the art. These additives include processing aids and performance aids such as crosslinking agents, natural and synthetic binders, plasticizers, softeners, foam-inhibiting agents, froth aids, flame retardants, dispersing agents, pH-adjusting components, sequestering or chelating agents, and other components.

In another aspect, the invention relates to a treated fibrous material. The treated fibrous material comprises at least one fiber and a cationic polymer latex described herein positioned on the fiber. If desired, the polymer may be applied to the fiber in the form of a powder. The composition may be deposited on the fiber by methods known to one skilled in the art.

For the purposes of the invention, the term "fiber" is to be broadly construed and may include single or multiple filaments that may be present in a variety of ways. One should appreciate that only a single fiber can be treated by the cationic polymer latex of the invention if so desired. The fibers used in the invention may encompass natural and/or synthetic fibers. For example, natural fibers include animal fibers (e.g., silk, wool); mineral fibers (e.g., asbestos); and vegetable-based fibers (e.g., cotton, flax, jute, and ramie). Cellulosic and wood fibers may also be used. Examples of synthetic fibers include those made from polymers such as polyamides, polyesters, acrylics, and polyolefins. Other examples of fibers include rayon and inorganic substances extruded in fibrous form such as glass, boron, boron carbide, boron nitride, carbon, graphite, aluminum silicate, fused silica, and metals such as steel. Recycled fibers using any of the above materials may also be employed. Mixtures of the above fibers may be used.

The treated fibrous material may have at least one polymeric layer deposited on the fiber so as to form a composite fibrous structure. Multiple polymer layers may be used as desired by one skilled in the art. As an example, anionic polymer latices may be deposited on the treated fibrous material to enhance specific properties of the treated fibrous material. Thus, unique fibers with specially modified surfaces can conceivably be made in accordance with the invention.

The invention also provides an article of manufacture comprising a substrate and a cationic polymer latex deposited and positioned thereon as defined herein. The cationic polymer latex may be in the form of a powder if so desired. For the purposes of the invention, the term "substrate" is to be broadly interpreted and include all those formed from inorganic materials, organic materials, and composites thereof. The substrate can encompass fibers, fillers and pigments as well as other organic and inorganic materials. Preferably, a fibrous substrate is employed. The term "fibrous substrate" is to be broadly interpreted to include the fibers described herein. The fibrous substrate may be present in the form of web, yarn and fabric. The fibrous substrate can be in the form of a textile substrate. For the purposes of the invention, the term "textile substrate" is similar to that defined in U.S. Patent No. 5,403,640 to Krishnan et al.. For example, "textile substrate" can be interpreted to encompass a fiber, web, yarn, thread, sliver, woven fabric, knitted fabric, non-woven fabric, upholstery fabric, tufted carpet and pile carpet formed from any of the fibers described herein. The article of manufacture can be made in accordance with known procedures. The invention also provides a coated material comprising a material having a cationic polymer latex deposited. For the purposes of the invention, the term material refers to, but is not limited to, a fiber, filler, particle, pigment and composites thereof. These materials may be organic, inorganic, or a composite of both as described herein.

Other layers of polymers may be deposited on the cationic polymer latex which is present in the article of manufacture to form a composite structure. For example, the deposited cationic latices can be followed by the deposition of anionic latices or other polymers to enhance specific properties of the article of manufacture. Unique fibers which comprise the fibrous substrate with specially modified surfaces can be made in accordance with the invention.

A multiple deposition process can also be used to make composite films that have applications in areas other than textile articles. For example, the cationic latices of the invention can also be used to make multilayer elastomeric gloves. Cellulosic structures can also be made by the cationic latices of the invention which encompasses cellulosic composites and heavy duty cellulosic structures. Examples of cellulosic composites include those relating to filtration, shoe insole, flooring felt, gasketing, as well as other applications. Heavy duty cellulosic structures include dunnage bags, and industrial wipes. Other areas of use for this technology include, but are not limited to, flocculants, wet and dry strength additives for papermaking, retention aids, cement modifications, dye fixation used redispersible powders.

The invention is advantageous in many respects. An especially desirable feature of the invention is that the cationic latices may be completely deposited on a substrate such that residual latex does not remain in the processing fluid medium, which is potentially advantageous from an environmental standpoint. The cationic latices can be preferentially deposited on a substrate that has a net negative charge, and can be deposited in a uniform manner which uses less latex (e.g., less than 5 percent). Preferably, the cationic latices can deposit on the substrate surface as a monolayer. The cationic latices may be formed by existing emulsion polymerization processes. Such processes advantageously allow for the preparation of high molecular weight polymers. The cationic polymers latices of the invention also obviate the need for retention aids and cationic surfactants. Most preferably, the cationic polymers latices are devoid of cationic surfactants. This is particularly desirable, since these materials are potentially toxic in aquatic environments. Thus, the polymer latex of the invention is more environmentally friendly. Moreover, if desired, the polymer latices may be devoid of conventional surfactants, e.g., nonionic surfactants. The latices are also clean. For the purpose of the invention, the term "clean" refers to the latices having preferably less than 0.1 percent coagulum and/or preferably less than 50 ppm grit on a 200 mesh screen and more preferably less than 10 ppm grit. The polymer latices of the invention also exhibit high performance properties.

The following examples are intended to illustrate the invention.

### Example 1

The cationic latex of the invention can be made by a batch or semicontinuous process. The procedure outlined below is for a batch process. A solution was made by dissolving 105 gms of methoxy polyethyleneglycol methacrylate, 30 gms of polymerizable surfactant (e.g., SAM 186N), 62.5 gms of N-methylol acrylamide (48% active), and 60 gms dimethylaminoethyl methacrylate in 2600 gms of deionised water. The pH of the solution was adjusted to about 4 with 36.5 gms hydrochloric acid (37% active) and this solution was then charged into a 1 gallon (3.8 liter) reactor. The reactor was purged several times with nitrogen and a mixture of 900 gms styrene and 405 gms butadiene was added into the reactor. The temperature was then raised to about 140°C and 6 gms of the cationic initiator Wako V-50 was injected into the reactor as a solution in 45 gms of deionised water. The reaction is continued until the monomer conversion is greater than 95 percent. The temperature is raised as needed to obtain a total reaction time of 9-11 hours. The latex may also be stripped to a desired content, usually to about 40 percent.

### Example 2

To a four necked 1-liter flask, 690 gms of deionized water (DW) and 12 gms DMAEMA was charged. The pH was adjusted to approximately 4.0 with concentrated hydrochloric acid (37% active). 12 gms MPEG 550, 3 gms SAM 186N, 6 gms Abex 2525 (50% active) was then added along with an initial monomer charge of 60 gms MMA and 60 gms BA. The temperature was raised to 70°C and 1.2 gms of Wako V-50 was then injected. After about 50 percent conversion of the initial monomer was achieved, the feeds were initiated. The feeds comprised: (1) 222 gms MMA and 174 gms BA which was fed over 5 hrs; (2) an aqueous feed of 60 gms DW, 30 gms MPEG 550, 37.5 gms NMA (48% active), and 9 gms SAM 186N which was fed over 3 hrs; (3) a cationic monomer feed of 12 gms DMAEMA, 7.3 gms HCl, and 60 gms DW that was fed over 3 hrs; and (4) a catalyst feed of 120 gms DW and 1.2 gms of Wako V-50 that was fed over 5.5 hrs. The temperature was gradually raised to 85°C over 6 hrs and the reaction was carried to complete conversion. The latex had a final solids content of 38.1 percent at a pH of 4.5. The coagulum in the final latex was negligible (i.e., less than 0.05 percent) and the grit in the latex was 28 ppm on a 200 mesh screen.

### Example 3

The procedure according to Example 2 was employed except that the monomer composition was changed. The latex had the following monomer composition (gms): STY/MMA/BA/DMAEMA/MPEG 550/NMA (48% active) = 60/300/156/24/42/37.5. The latex had a final solids content of 39 percent at a pH of 4.4. The coagulum in the latex was negligible and the grit on a 200 mesh screen was 97 ppm.

### Example 4

The procedure according to Example 3 was employed except that the monomer composition was different. The latex had the following monomer composition (gms): STY/BA/DMAEMA/MPEG 550/NMA (48% active) = 432/96/24/30/37.5. Also, this recipe had no Abex 2525 but instead used 15 gms of SAM 186N in the aqueous surfactant feed in addition to 3 gms in the initial batch. Also, the level of V-50 initiator was increased from 1.2 gms to 1.8 gms in the catalyst feed. The latex had a final solids content of 40.3 percent at a pH of 4.3. The coagulum in the latex was negligible and the grit on a 200 mesh screen was 48 ppm.

### Example 5

The process is a batch process and is similar to that described in Example 1 with the following monomer composition (gms): DMAEMA/NMA (48% active)/AN/STY/BD/MPEG 550 = 75/62.5/255/150/915/75. In addition, the latex had 37.5 gms of polymerizable surfactant (SAM 186-N). The final latex before stripping had a solids content of 34.3 percent and a pH of 4.8 at a viscosity of 44 cps. The latex was very clean and had no coagulum and the grit on a 200 mesh screen was negligible (less than 2 ppm). This latex also did not use conventional surfactant, e.g., Abex 2525.

### Examples 6-11

### Comparative Examples

Latices were prepared according to R.H.Ottewill, A.B.Schofield, J.A.Waters, N.St.J. Williams "Preparation of core-shell polymer colloid particles by encapsulation", Colloid Polym Sci 275: 274-283, (1997). Ottewill et al. is primarily interested in looking at forming core-shell latex particles by encapsulation of a cationic latex with an anionic latex. Example 6 represents a latex prepared according to Ottewill et al. Examples 7-11 represent variations of the procedure of Example 6. Nonetheless, none of the latices that were prepared according to Examples 6-11 were clean (as defined herein) and commercially viable.

### Example 6

A latex according to a procedure proposed by Ottewill et al. was formed from the following recipe:

| Ingredient | gms |
|---|---|
| n-butyl methacrylate | 543 |
| Wako V-50 | 4.8 |
| polyethyleneglycol methacrylate | 57 |
| (Bisomer S10W)(W=2000) | |
| sodium chloride | 18 |
| deionized water | 5400 |

The latex was polymerized at 70°C. When the experiment was repeated according to Ottewill, the latex had a final solids content of 9.9 percent, a pH of 5.0, a coagulum of 2.6 percent and grit on a 200 mesh screen of 86 ppm. The particle size of the latex was 603 nm.

### Example 7

The procedure of Example 6 was repeated except that MPEG 550 (MW=550) replaced S10W. A latex with a much higher coagulum, about 23.4 percent, resulted.

### Example 8

The procedure of Example 6 was repeated except that 1080 gms of deionized water was employed instead of 5400. This change was carried out in order to increase the solids content of the latex, which was between 36 and 37 percent Nonetheless, the entire latex coagulated.

### Example 9

The procedure of Example 6 was repeated at a much lower salt concentration, because salt concentration is believed to affect stability and particle size. Using 1.2 gms sodium chloride in the above recipe, a latex of 1.6 percent coagulum with a particle size of approximately 283 nm, and grit on a 200 mesh screen of 58 ppm resulted.

### Example 10

The procedure of Example 9 was repeated using 1080 gms water to attempt to achieve a latex with a higher solids content. Although the latex achieved a higher solids content (33.3 percent), the latex had 1.8 percent coagulum and grit on a 200 mesh screen of 84 ppm.

### Example 11

The procedure outlined in Example 6 was employed, except that the following recipe was used:

| Ingredient | gms |
|---|---|
| deionized water | 1080 |
| Wako V-50 | 4.8 |
| styrene | 372 |
| butadiene | 171 |
| Bisomer S10W | 57 |
| sodium chloride | 1.2 |

The composition was polymerized at 70°C. This recipe is designed for comparison to the procedure for making a styrene/butadiene latex described in Example 1. When this recipe is used using the procedure of Example 6, it results in complete coagulation of the latex, i.e., the entire latex destabilized.

### Example 12

### Addition of Cationic Monomer

The procedure of Example 11 was repeated except that 24 gms of a cationic monomer (e.g., dimethyl aminoethyl methacrylate methyl chloride quaternary, FM1 Q75MC) is added in place of 24 gms of the butadiene charge. The resulting latex is much cleaner and there is about 2.5 percent coagulum and 96 ppm grit on a 200 mesh screen at a final solids of 34.4 percent Thus, the addition of a cationic monomer to an Ottewill, et al recipe significantly improves its stability.

### Example 13

The procedure of Example 11 was repeated using 3 gms salt and cationic monomer described in Example 12 and MPEG 550 in place of Bisomer S10W. The latex has trace amounts of coagulum and 14 ppm grit at a solids content of 34.9 percent Thus, the use of steric stabilizing monomer clearly helps to significantly improve the stability and cleanliness of the latex.

### Examples 14-17

### Cationic Polymer Latices

Examples 14-17 represent various cationic polymer latices. These examples are intended to show the importance of the steric stabilizing mechanism and its ability to impart stability to the latex. One can use polymerizable components such as, for example, MPEG 550 and SAM 186N or conventional nonionic surfactants such as, for example, Abex 2525.

### Example 14

A latex was made according to the procedure outlined in Example 1 with the following monomer composition (gms): NMA (48% active) /STY/BD/DMAEMA= 62.5/930/480/60. The temperature of the polymerization was 70°C. The resulting latex had a 4.15 percent coagulum and a grit level of 130 ppm on a 200 mesh screen at a solid content of 32.4 percent. The latex is believed to be not clean without employing steric stabilizing monomers such as MPEG 550 and SAM 186N.

### Example 15

The procedure according to Example 14 was repeated except that the butadiene level was reduced to 420 gms, 60 gms of SAM 186N was added, and 7.5 gms of Abex 2525 (50% active), a conventional non-ionic surfactant, was employed. The resulting latex had no coagulum and 28 ppm grit at a solids content of 33.6 percent.

### Example 16

The procedure according to Example 15 was repeated using half the amount of SAM 186 N. The resulting latex was not as clean and had a coagulum of 0.7 percent and grit of 114 ppm at a solids content of 33.8 percent.

### Example 17

The procedure according to Example 16 was repeated using 105 gms of MPEG 550 and 345 gms of butadiene without the Abex 2525. The resulting latex is much cleaner with only 0.2 percent coagulum and 26 ppm grit at a solids level of 34.1 percent. The butadiene level in this case was set to compensate for the additional MPEG 550.

### Examples 18-20

### Effect of Conventional Surfactants on Stability of Polymer Latices

Examples 18-20 illustrate the effect of using a conventional nonionic surfactant on latex stability. While helpful, these materials may not be adequate in the amounts used to impart stability on their own. The latices are believed to be more stable when used in conjunction with the polymerizable surfactants as shown in the earlier examples,

### Example 18

A latex was made according to the procedure outlined in Example 1 with the following monomer composition (gms): NMA (48% active)/STY/BD/DMAEMA =62.5/930/480/60. 30 gms of Abex 2525 (50% active) was employed, along with 7.5 gms of initiator Wako V-50.

The temperature of the polymerization was 70°C. The resulting latex had a 2.6 percent coagulum and a solids content of 33.5 percent.

### Example 19

The procedure according to Example 18 was carried out except that the level of Abex 2525 was increased to 45 gms. The resulting latex was still not clean.

### Example 20

The procedure according to Example 18 was carried out except that dimethylaminoethyl methacrylate was replaced by its quaternary version (FM1Q75MC), The resulting latex produced less coagulum (1.27 percent), but was still considered unacceptable.

### Example 21

A latex was made according to the procedure of Example 4 with the following monomer composition (gms): FM1Q75MC/NMA (48% active)/STY=30/37.5/552.

The recipe was polymerized at 70°C. The latex made according to this recipe had a final solids content of 26.1 percent, a pH of 5, and a viscosity of 18 cps. The coagulum amount was 2.39 percent. This example is intended to demonstrate that without employing steric stabilizing monomers, a clean latex could not be attained even at this solids content.

### Examples 22-25

### Comparative Data - Beater Addition Process

Table 1 illustrates comparative data of various paper samples having latex added thereon via a beater addition process. Example 22 represents a sample without latex. Example 23 represents a sample with a commercially available anionic latex having a 52/48 styrene to butadiene ratio. Examples 24 and 25 represent samples using cationic latices prepared according to the procedure of Example 1. As seen, the samples using the latices of the invention generally display superior physical properties to Examples 22 and 23.

### Examples 26-28

### Comparative Data - Saturation Process

Table 2 illustrates comparative data of various paper samples having latex added thereon via a saturation process. Example 26 represents a sample with a commercially available anionic latex having a 55/45 styrene to butadiene ratio. Examples 27 and 28 represent samples using cationic latices prepared according to the procedure of Example 1. As seen, the samples using the latices of the invention exhibit good physical properties relative to Example 26 while employing a much lower amount of latex.

### Examples 29-33

### Comparative Data - Saturation Process

Table 3 illustrates comparative data of various paper samples having latex added thereon via a saturation process. Example 29 represents a sample without latex. Examples 30 and 31 represent samples using commercially available anionic latices having 40/60 and 55/45 styrene to butadiene ratios respectively. Examples 32 and 33 represent samples using cationic latices prepared according to the procedure of Example 1. As seen, the samples using the latices of the invention exhibit superior physical properties relative to Examples 29 through 31 while employing a much lower amount of latex.

**TABLE 1**

| CATIONIC LATICES | | | | |
|---|---|---|---|---|
| Comparison with Anionic Latices - Beater Addition Process | | | | |
| Example | (22) dry control | Styrene/Butadiene 52/48 (23) | Reichhold Cationic (24) | Reichhold Cationic (25) |
| Tg of polymer, degree C | | -19 | -31 | -31 |
| Latex Add-on, % | 0 | 10 | 5 | 10 |
| Tensile, lb. (kg) | 32.3 (14.68) | 40.9 (18.59) | 112.1 (509.5) | 130.7 (59.4) |
| Tensile, psi (MPa) | 807 (5.56) | 1021 (7.04) | 2799 (19.3) | 3268 (22.5) |
| Tensile Index | --- | 102 | 560 | 327 |
| Wet Tensile - 1 hour, psi (MPa) | --- | 179 (1.23) | 1219 (8.40) | 1983 (13.67) |
| Wet Tensile - 6 hour, psi (MPa) | --- | 179 (1.23) | 1012 (6.98) | 1405 (9.69) |
| Wet Tensile - 24 hour, psi (MPa) | --- | 166 (1.14) | 995 (6.86) | 1133 (7.81) |
| Notes: 1. 100% Softwoods - bleached sulfite. | | | | |
| 2. Tensile Index is PSI/Latex Add-on. | | | | |
| 3. Dry Control is Substrate without Latex. | | | | |

**TABLE 2**

| CATIONIC LATICES | | | |
|---|---|---|---|
| Comparison OF Wet Strength with Anionic Latices - Saturation Process | | | |
| Example | Styrene/Butadiene 55/45 (26) | Reichhold Cationic (27) | Reichhold Cationic (28) |
| Tg of polymer, degree C | -5 | 8 | -31 |
| Latex Add-on, % | 31.3 | 3.6 | 5.7 |
| Tensile, lb. (kg) | 82.8 (37.6) | 81.2 (36.9) | 86.1 (39.1) |
| Tensile, psi (MPa) | 2267 (15.6) | 2881 (19.9) | 3351 (23.1) |
| Tensile Index | 72 | 800 | 588 |
| Wet Tensile - 1 hour, psi (MPa) | 787 (5.4) | 712 (4.9) | 1374 (9.5) |
| Wet Tensile - 6 hour, psi (MPa) | 909 (6.3) | 652 (4.5) | 1150 (7.9) |
| Notes: 1. 100% Softwoods - bleached sulfite. | | | |
| 2. Tensile Index is PSI/Latex Add-on. | | | |

**TABLE 3**

| CATIONIC LATICES | | | | | |
|---|---|---|---|---|---|
| Comparison with Anionic Latices - Saturation Process | | | | | |
| Example | (29) dry control | Styrene/Butadiene 40/60 (30) | Styrene/Butadiene 55/45 (31) | Reichhold Cationic (32) | Reiohhold Cationic (33) |
| Tg of polymer, degree C | | -36 | -5 | 5 | 8 |
| Latex. Add-on, % | 0 | 31.3 | 16.3 | 5.4 | 5.9 |
| Basis Weight, lb/yd2 (kg/m2) | 0.9 (0.49) | 1.18 (0.64) | 1.05 (0.57) | 0.95 (0.52) | 0.95 (0.52) |
| Density | 0.55 | 0.59 | 0.56 | 0.54 | 0.54 |
| Tensile, lb. (kg) | 39.24 (17.84) | 83.11 (37.78) | 80.9 (36.78) | 112.5 (51.14) | 128.9 (58.59) |
| Elongation, % | 2.4 | 10.3 | 7 | 6.5 | 6.5 |
| Tensile, psi (MPa) | 1060 (7.3) | 1808 (12.47) | 1759 (12.13) | 3136 (21.62) | 3485 (24.03) |
| Tensile index | --- | 58 | 108 | 581 | 591 |
| Notes: 1. Dry Control is substrate without latex. | | | | | |
| 2. Tensile Index is PSI/Latex Add-on. | | | | | |
| 3. 50/50 fiber blend of softwoods. | | | | | |

## Claims

1. A cationic polymer latex formed by emulsion polymerisation comprising:
at least one ethylenically unsaturated monomer;
an ethylenically unsaturated cationic monomer;
a monomer possessing alkoxylated functionality incorporated into said cationic polymer latex to provide steric stabilization; and
a free radical initiator.

2. The latex according to Claim 1 wherein said cationic polymer latex is devoid of cationic surfactant and has a solids content of no less than 35 weight percent.

3. The latex according to Claim 1 or 2, wherein said ethylenically unsaturated monomer is selected from vinyl aromatic monomers, olefins, aliphatic conjugated diene monomers, non-aromatic unsaturated mono- or dicarboxylic ester monomers, monomers based on the half ester of an unsaturated dicarboxylic acid monomer, unsaturated mono- or dicarboxylic acid monomers and derivatives thereof, nitrogen-containing monomers, vinyl acetate, vinyl ester monomers, and mixtures thereof.

4. The latex according to any one of Claims 1, 2 or 3, wherein said ethylenically unsaturated cationic monomer comprises a heteroatom selected from nitrogen, phosphorus and sulphur.

5. The latex according to any one of Claims 1 to 4 wherein said ethylenically unsaturated cationic monomer is an amine monomer.

6. The latex according to any of the preceding Claims and comprising:
from 70 to 99 weight percent of at least one ethylenically unsaturated monomer;
from 0.5 to 15 weight percent of an ethylenically unsaturated cationic monomer; and
from 0.5 to 15 weight percent of a monomer possessing alkoxylated functionality incorporated into said cationic polymer latex.

7. The latex according to any of the preceding Claims, wherein said monomer possessing alkoxylated functionality comprises a monomer having a formula selected from:
CH₂=C(R)COO(CH₂CHR'O)ₙR"
wherein R, R', and R" are each selected from the group consisting of H, and C₁-C₄ alkyl, and wherein 1 ≤ n ≤ 30; and
CH₂=C(R)COO(CH₂CH₂O)ₙ(CH₂CHR'O)ₘR"
wherein R, R', and R" are each selected from the group consisting of H and C₁-C₄ alkyl, 1 ≤ n ≤ 15, and 1 ≤ m ≤ 15.

8. The latex according to any of the preceding Claims wherein said monomer possessing alkoxylated functionality is selected from:
(a) CH₂=C(R)COO(CH₂CHR'O)ₙ, R", where R=H, C₁-C₄ alkyl; and R'= H, C₁-C₄ alkyl, and R"= H, C₁-C₄ alkyl, and n=1-30;
(b) CH₂=C(R)COO(CH₂CH₂O)ₙ (CH₂CHR'O)ₘ R", where R= H, C₁-C₄ alkyl, and R'= H, C₁-C₄ alkyl, and R"= H, C₁-C₄ alkyl, n and m each may range from 1-15;
(c) CH₂=C(R)COO(CH₂CHR'O)ₙ (CH₂CH₂O)ₘ R", where R= H, C₁-C₄ alkyl, and R'=H, C₁-C₄ alkyl and R"= H, C₁-C₄ alkyl, n and m = 1-15; and
(d) mixtures of (a) and (b),
and said latex is devoid of cationic surfactants.

9. The latex according to Claim 8, wherein R, R', and R" in component (b) or component (c) are each CH₃.

10. A treated fibrous material comprising at least one fibre and a latex according to any one of Claims 1 to 6, said latex being deposited uniformly on said at least one fibre.

11. The treated fibrous material according to Claim 10, wherein said at least one fibre is selected from cellulose, wood, and mixtures thereof.

12. The treated fibrous material according to claim 10 or 11, further comprising at least one polymeric layer positioned on said at least one fibre.

13. An article of manufacture comprising a substrate and a latex according to any of Claims 1 to 6, said latex being deposited uniformly on said substrate.

14. The article of manufacture according to Claim 13, wherein said substrate comprises at least one material selected from fibres, fillers, organic materials, and inorganic materials.

15. The article of manufacture according to Claim 13 wherein said substrate is a fibrous substrate comprising fibres selected from cellulose fibres, wood fibres, and mixtures thereof.

16. The article of manufacture according to any one of Claims 13 to 15, further comprising at least one polymeric layer positioned on said fibrous substrate.

17. The article of manufacture according to any one of Claims 13 to 16, wherein said article of manufacture is an elastomeric glove.

18. The article of manufacture according to any one of Claims 13 to 16 wherein said article of manufacture is a cellulosic structure.

19. The article of manufacture according to any one of Claims 13 to 18 wherein said latex is present as a powder.

## Patentansprüche

1. Latex eines kationischen Polymers, gebildet durch Emulsions-Polymerisation, umfassend:
- wenigstens ein ethylenisch ungesättigtes Monomer;
- ein ethylenisch ungesättigtes kationisches Monomer;
- ein Monomer, das Alkoxy-Funktionalität besitzt und in dem Latex des kationischen Polymers unter Schaffung einer sterischen Stabilisierung eingebaut wird; und
- einen Initiator zur Bildung freier Radikale.

2. Latex nach Anspruch 1, worin der Latex eines kationischen Polymers frei von kationischem Tensid ist und einen Feststoff-Gehalt von nicht weniger als 35 Gew.-% aufweist.

3. Latex nach Anspruch 1 oder 2, worin das ethylenisch ungesättigte Monomer gewählt ist aus Vinyl-aromatischen Monomeren, Olefinen, aliphatischen konjugierten Dien-Monomeren, nicht-aromatischen ungesättigten Mono- oder Dicarbonsäureester-Monomeren, Monomeren auf der Basis des Halbesters eines ungesättigten Dicarbonsäure-Monomers, ungesättigten Mono- oder Dicarbonsäure-Monomeren und Derivaten davon, Stickstoff enthaltenden Monomeren, Vinylacetat, Vinylester-Monomeren und Mischungen daraus.

4. Latex nach irgendeinem der Ansprüche 1, 2 oder 3, worin das ethylenisch ungesättigte kationische Monomer ein Hetero-Atom umfasst, das gewählt ist aus Stickstoff, Phosphor und Schwefel.

5. Latex nach irgendeinem der Ansprüche 1 bis 4, worin das ethylenisch ungesättigte kationische Monomer ein Amin-Monomer ist.

6. Latex nach irgendeinem der vorangehenden Ansprüche und umfassend:
- 70 bis 99 Gew.-% wenigstens eines ethylenisch ungesättigten Monomers;
- 0,5 bis 15 Gew.-% eines ethylenisch ungesättigten kationischen Monomers; und
- 0,5 bis 15 Gew.-% eines Monomers, das Alkoxy-Funktionalität besitzt und in den Latex eines kationischen Polymers eingearbeitet ist.

7. Latex nach irgendeinem der vorangehenden Ansprüche, worin das Monomer, das Alkoxy-Funktionalität besitzt, ein Monomer mit einer Formel umfasst, die gewählt ist aus:
CH₂=C(R)COO(CH₂CHR'O)ₙR",
worin R, R' und R" jeweils gewählt sind aus der Gruppe, die besteht aus H und C₁- bis C₄-Alkyl, und worin 1 ≤ n ≤ 30 ist; und
CH₂=C(R)COO(CH₂CH₂O)ₙ(CH₂CHR'O)ₘR",
worin R, R' und R" jeweils gewählt sind aus der Gruppe, die besteht aus H und C₁- bis C₄-Alkyl, 1 ≤ n ≤ 15 und 1 ≤ m ≤ 15 sind.

8. Latex nach irgendeinem der vorangehenden Ansprüche, worin das Monomer, das Alkoxy-Funktionalität besitzt, gewählt ist aus :
(a) CH₂=C(R)COO(CH₂CHR'O)ₙR",
worin R=H, C₁- bis C₄-Alkyl; und R'=H, C₁- bis C₄-Alkyl sind; und R"=H, C₁- bis C₄-Alkyl ist; und n=1 bis 30 ist;
(b) CH₂=C(R)COO(CH₂CH₂O)ₙ(CH₂CHR'O)ₘR",
worin R=H, C₁- bis C₄-Alkyl; und R'=H, C₁- bis C₄-Alkyl sind; und R"=H, C₁- bis C₄-Alkyl ist; und n und m jeweils im Bereich von 1 bis 15 liegen können;
(c) CH₂=C(R)COO(CH₂CHR'O)ₙ (CH₂CHR'O)ₘR",
worin R=H, C₁- bis C₄-Alkyl; und R'=H, C₁- bis C₄-Alkyl sind; und R"=H, C₁- bis C₄-Alkyl ist; und n und m 1 bis 15 sind; und
(d) Mischungen von (a) und (b);
und der Latex frei von kationischen Tensiden ist.

9. Latex nach Anspruch 8, worin R, R' und R" in Komponente (b) oder Komponente (c) jeweils CH₃ sind.

10. Behandeltes faseriges Material, umfassend wenigstens eine Faser und einen Latex nach irgendeinem der Ansprüche 1 bis 6, wobei der Latex einheitlich auf wenigstens einer Faser abgeschieden ist.

11. Behandeltes faseriges Material nach Anspruch 10, worin die wenigstens eine Faser gewählt ist aus Cellulose, Holz und Mischungen daraus.

12. Behandeltes faseriges Material nach Anspruch 10 oder 11, weiter umfassend wenigstens eine Polymer-Schicht, die auf der wenigstens einen Faser positioniert ist.

13. Industriell hergestellter Gegenstand, umfassend ein Substrat und einen Latex nach irgendeinem der Ansprüche 1 bis 6, wobei der Latex einheitlich auf dem Substrat abgeschieden ist.

14. Industriell hergestellter Gegenstand nach Anspruch 13, worin das Substrat wenigstens ein Material umfasst, das gewählt ist aus Fasern, Füllstoffen, organischen Materialien und anorganischen Materialien.

15. Industriell hergestellter Gegenstand nach Anspruch 13, worin das Substrat ein faseriges Substrat ist, das Fasern umfasst, die gewählt sind aus Cellulose-Fasern, Holz-Fasern und Mischungen daraus.

16. Industriell hergestellter Gegenstand nach irgendeinem der Ansprüche 13 bis 15, weiter umfassend wenigstens eine polymere Schicht, die auf dem faserigen Substrat angeordnet ist.

17. Industriell hergestellter Gegenstand nach irgendeinem der Ansprüche 13 bis 16, worin der industriell hergestellte Gegenstand ein elastomerer Handschuh ist.

18. Industriell hergestellter Gegenstand nach irgendeinem der Ansprüche 13 bis 16, worin der industriell hergestellte Gegenstand eine Cellulose-artige Struktur ist.

19. Industriell hergestellter Gegenstand nach irgendeinem der Ansprüche 13 bis 18, worin der Latex als Pulver vorliegt.

## Revendications

1. Latex de polymère cationique formé par polymérisation en émulsion, comprenant :
- au moins un monomère à insaturation éthylénique ;
- un monomère cationique à insaturation éthylénique ;
- un monomère possédant une fonctionnalité alcoxylée incorporée dans ledit latex de polymère cationique pour fournir une stabilisation stérique ; et
- un amorceur de radicaux libres.

2. Latex selon la revendication 1, dans lequel ledit latex de polymère cationique est dépourvu d'agent tensio-actif cationique et possède une teneur en matières solides de pas moins de 35 pour cent en poids.

3. Latex selon l'une des revendications 1 ou 2, dans lequel ledit monomère à insaturation éthylénique est choisi parmi les monomères vinyl aromatiques, les oléfines, les monomères diènes conjugués aliphatiques, les monomères esters mono- ou dicarboxyliques insaturés non aromatiques, les monomères à base de l'hémi-ester d'un monomère acide dicarboxylique insaturé, les monomères acides mono- ou dicarboxyliques insaturés et leurs dérivés, les monomères contenant de l'azote, l'acétate de vinyle, les monomères esters vinyliques et leurs mélanges.

4. Latex selon l'une quelconque des revendications 1, 2 ou 3, dans lequel ledit monomère cationique à insaturation éthylénique comprend un hétéroatome choisi parmi l'azote, le phosphore et le soufre.

5. Latex selon l'une quelconque des revendications 1 à 4, dans lequel ledit monomère cationique à insaturation éthylénique est un monomère amine.

6. Latex selon l'une quelconque des revendications précédentes et comprenant :
- de 70 à 99 pour cent en poids d'au moins un monomère à insaturation éthylénique ;
- de 0,5 à 15 pour cent en poids d'un monomère cationique à insaturation éthylénique ; et
- de 0,5 à 15 pour cent en poids d'un monomère possédant une fonctionnalité alcoxylée incorporée dans ledit latex de polymère cationique.

7. Latex selon l'une quelconque des revendications précédentes, dans lequel ledit monomère possédant une fonctionnalité alcoxylée comprend un monomère ayant une formule choisie parmi :
CH₂=C(R)COO(CH₂CHR'O)ₙR"
dans laquelle R, R' et R" sont chacun choisis dans le groupe constitué par H et alkyle en C₁-C₄ et dans laquelle 1 ≤ n ≤ 30 ; et
CH₂=C(R)COO(CH₂CH₂O)ₙ(CH₂CHR'O)ₘR"
dans laquelle R, R' et R" sont chacun choisis dans le groupe constitué par H et alkyle en C₁-C₄, 1 ≤ n ≤ 15 et 1 ≤ m ≤ 15.

8. Latex selon l'une quelconque des revendications précédentes, dans lequel ledit monomère possédant une fonctionnalité alcoxylée est choisi parmi :
(a) CH₂=C(R)COO(CH₂CHR'O)ₙ R", où R=H, alkyle en C₁-C₄ ; et R' = H, alkyle en C₁-C₄ et R" = H, alkyle en C₁-C₄ et n =1-30 ;
(b) CH₂=C(R)COO(CH₂CH₂O)ₙ (CH₂CHR'O)ₘ R", où R = H, alkyle en C₁-C₄ et R' = H, alkyle en C₁-C₄, et R" = H, alkyle en C₁-C₄, n et m peuvent chacun se situer dans la plage de 1-15 ;
(c) CH₂=C(R)COO(CH₂CHR'O)ₙ (CH₂CH₂O)ₘ R", où R = H, alkyle en C₁-C₄ et R' = H, alkyle en C₁-C₄ et R" = H, alkyle en C₁-C₄, n et m = 1-15 ; et
(d) des mélanges de (a) et (b),
et ledit latex est dépourvu d'agents tensio-actifs cationiques.

9. Latex selon la revendication 8, dans lequel R, R' et R" dans le composant (b) ou le composant (c) représentent chacun CH₃.

10. Matière fibreuse traitée comprenant au moins une fibre et un latex tel que défini à l'une quelconque des revendications 1 à 6, ledit latex étant déposé de façon uniforme sur ladite au moins une fibre.

11. Matière fibreuse traitée selon la revendication 10, dans laquelle ladite au moins une fibre est choisie parmi la cellulose, le bois et leurs mélanges.

12. Matière fibreuse traitée selon l'une des revendications 10 ou 11, comprenant en outre au moins une couche polymère positionnée sur ladite au moins une fibre.

13. Article de fabrication comprenant un substrat et un latex tel que défini à l'une quelconque des revendications 1 à 6, ledit latex étant déposé de façon uniforme sur ledit substrat.

14. Article de fabrication selon la revendication 13, dans lequel ledit substrat comprend au moins un matériau choisi parmi les fibres, les charges, les matières organiques et les matières inorganiques.

15. Article de fabrication selon la revendication 13, dans lequel ledit substrat est un substrat fibreux comprenant des fibres choisies parmi les fibres de cellulose, les fibres de bois et leurs mélanges.

16. Article de fabrication selon l'une quelconque des revendications 13 à 15, comprenant en outre au moins une couche polymère positionnée sur ledit substrat fibreux.

17. Article de fabrication selon l'une quelconque des revendications 13 à 16, dans lequel ledit article de fabrication est un gant élastomère.

18. Article de fabrication selon l'une quelconque des revendications 13 à 16, dans lequel ledit article de fabrication est une structure cellulosique.

19. Article de fabrication selon l'une quelconque des revendications 13 à 18, dans lequel ledit latex est présent sous la forme d'une poudre.
